

# UNITED STATES PATENT OFFICE.

JOHN D. CHEEVER, OF NEW YORK, N. Y.

## COVER FOR FLOORS AND FOR OTHER PURPOSES.

SPECIFICATION forming part of Letters Patent No. 285,343, dated September 18, 1883.

Application filed August 27, 1883. (No specimens.)

*To all whom it may concern:*

Be it known that I, JOHN D. CHEEVER, a citizen of the United States, residing at New York, in the county of New York and State of New York, have invented certain new and useful Improvements in the Manufacture of Covers for Floors and for other Purposes, by which flexible and durable imitations of porcelain, mosaic work, marble, slate, and wood tiles are made; and I do hereby declare the following to be a full, clear, and exact description of the invention, such as will enable others skilled in the art to which it appertains to make and use the same.

15 Flexible covers for floors are made by spreading on sheets of canvas, burlaps, and paper various plastic water-proof mixtures, and after the coatings are sufficiently set, dried, or hardened designs in colors are printed on them by 20 means of engraved wood blocks and paints composed of drying-oils and colored pigments. As these colors and the designs they form are superficial, they soon wear off at those parts most exposed and conspicuous, leaving only a 25 mottled unsightly surface.

25 To remedy these defects and provide a durable body with improved execution of designs or patterns which will not become erased nor altered before the whole fabric has been 30 destroyed are the objects of my invention.

The plastic material I employ is the product 35 prepared by the processes fully described in United States Letters Patent granted to me March 7, 1882, numbered 254,465. The product is formed by the chemical action of sub-chloride or protochloride of sulphur or mixtures of siccative oils with what is called by natives of Central America "pickum gum" and products derived from petroleum, as vaseline. It is an elastic and enduring substance, 40 which is ground or masticated with organic and mineral powders—such as cork, ivory-black, zinc-white, chrome-yellow, ultramarine, vermillion, red lead, and other like pigments—and then calendered or formed into sheets by the same provisions and manipulations used and practiced in the manufacture of caoutchouc. The sheets, made of every color 45 and tint, having the coloring-pigments uniformly mixed throughout their length and

thickness, are cut or stamped into pieces of shapes required for adjustment to form desired patterns or designs. The parts are joined firmly at their edges by a strong and durable water-proof cement.

55 The whole fabric, when completed, may be attached on one side to canvas, burlaps, prepared paper, or other suitable sheets by cement of the same qualities as that used for joining the edges of the sections.

60 A good cement is made by dissolving eighty parts of gutta-percha and twenty parts of caoutchouc in bisulphide of carbon, benzole, or naphtha.

65 The manufacture of the fabrics may be conveniently and more economically carried on by first joining the smaller pieces into sections of an area convenient to handle and then arranging these so as to complete a large sheet of required dimensions. While the work progresses a warm roller, used by a hand of the operator, is employed to hasten the volatilization of the solvent of the cement, and to insure 70 perfect adhesion of the parts and uniformity of the whole surface. Finally, the sheets may 75 be rolled into scrolls for convenience of transportation.

Although I have confined the description of my improvement to the use of the product described in the Letters Patent designated, I do 80 not desire to limit my claim specially to its use, as other plastic compounds capable of being ground with colored pigments and calendered may be substituted for it.

Having thus described my invention, what I 85 claim, and desire to secure by Letters Patent, is—

A flexible cover for floors and for other purposes, made by cutting small sections from sheets of plastic compounds of various colors, having colored pigments throughout their thickness, and cementing the pieces together, so as to form a sheet resembling porcelain, mosaic work, marble, slate, and wood tiles.

In testimony whereof I affix my signature in 95 presence of two witnesses.

JOHN D. CHEEVER.

Witnesses:

W. L. CANDEE,  
VICTOR E. BURKE.